

## UNITED STATES PATENT OFFICE

2,161,057

## BRAZING ALLOY

Philip R. Kalischer, Wilkinsburg, Pa., assignor to Westinghouse Electric & Manufacturing Company, East Pittsburgh, Pa., a corporation of Pennsylvania

No Drawing. Application March 31, 1939,  
Serial No. 265,228

4 Claims. (Cl. 75—153)

This invention relates generally to alloys and more particularly to brazing alloys.

Different brazing alloys have been produced heretofore, but they have not been altogether satisfactory in that they lack some of the characteristics initially desired in the alloy or as applied. For many applications, it is desired that the brazing alloys have low flow points of 725° C. and preferably lower than 700° C. In addition to the low flow points, the alloys should be ductile as applied or as fused in a joint, the ductility preferably approaching that of the well known 50% silver solders. Further, the alloy should have the characteristics of wetting metal parts without the use of a flux and of adhering to ferrous and non-ferrous metals.

An object of this invention is to provide a copper phosphorus brazing alloy having improved characteristics.

A more specific object of this invention is to provide a brazing alloy of copper, phosphorus and antimony having a low flow point, ductility as fused and the ability to adhere to non-ferrous metals and alloys.

Other objects of this invention will be apparent from the following description and the appended claims.

The alloy of this invention comprises antimony in an amount varying approximately from 1% to 6%, phosphorus varying approximately from 4% to 10% and the balance substantially all copper. In a preferred embodiment of the invention, the alloying elements are present in an amount ranging from 4 to 8% of phosphorus and from 5% to 4% of antimony with the balance substantially all copper.

In producing this brazing alloy, it is found that the antimony addition is very effective in lowering the flow point of the alloy without detrimentally affecting its ductility. In a number of cases it is found that the alloys whose contents fall within the ranges given hereinbefore where antimony is employed in place of the part of the phosphorus of the alloy, have a greater ductility than corresponding alloys which have a phosphorus content equal to the antimony plus phosphorus content of the alloy of this invention.

As illustrative of the effect of antimony additions on the flow point of the resulting copper-phosphorus-antimony alloy, reference may be had to the following table from which it is apparent that the antimony inclusions, both as additions to copper and phosphorus and as substitutions for part of the phosphorus content of

such alloys, have a definite effect in reducing the flow point of the resulting alloy.

| Alloy No. | Percent Sb | Percent P | Percent Cu | Flow point, °C. |
|-----------|------------|-----------|------------|-----------------|
| 15        | —          | 5         | 95         | 911             |
| 11        | —          | 7         | 93         | 832             |
| 16        | 0.5        | 7         | 92.5       | 724             |
| 12        | 1.0        | 6         | 93         | 704             |
| 13        | 2.0        | 6         | 92         | 685             |
| 14        | 4.0        | 6         | 90         | 679             |
| 18        | 3.0        | 4         | 93         | 716             |
| 20        | 2.0        | 5         | 93         | 704             |

The relationship given in the table has been found over a wide range of alloy compositions where the antimony plus phosphorus content in the copper base is from 5% to 10% of the whole. In practice, it is found that the best combination of characteristics of the alloy is obtained where the phosphorus plus antimony content is from 7% to 8% with the antimony present in amounts from .5 up to 4%, the resulting alloy having a low flow point, high ductility and extremely good self-fluxing characteristics. As employed in this description, the term "flow point" means the lowest temperature at which the alloy is completely fluid and as applied to the alloys of this invention, is also the melting point of the alloys, it being found that they have a very sharp melting point, the individual alloys having no melting range. The alloy identified in the table as No. 13 is of unusual value having a flow point below 700° C. while having a ductility far greater, as determined by bending a brazing joint, than the ductility obtained with a copper base alloy containing only 7% of phosphorus. In addition, this alloy adheres well to non-ferrous metals, no flux being necessary.

The copper-phosphorus-antimony alloys of this invention may be prepared by process analogous to those known to the art for the manufacture of other alloys. Thus a melt of copper and phosphorous having the desired phosphorus content may be made to which the antimony in the correct proportions may be added or the antimony and copper may be melted together, after which the phosphorus may be added in the correct proportions. The resulting alloy can be cast, and fabricated to a desired shape or form, or may be prepared for use as a powdered alloy. Whether employed in the solid form or in the powdered form, strong, dense and ductile welds are formed with non-ferrous metals and without any fluxing agent, since the resulting alloy has

self-fluxing characteristics with the ability to wet non-ferrous metals.

Although this invention has been described with reference to a particular embodiment, it is, of course, not to be limited thereto except insofar as is necessitated by the prior art and the scope of the appended claims.

I claim as my invention:

1. A brazing alloy comprising from 4% to 10% of phosphorus and from .1% to 6% of antimony with the balance substantially all copper.

2. A brazing alloy containing from 4% to 8%

of phosphorus and from .5% to 4% of antimony with the balance substantially all copper.

3. A brazing alloy composed of about 6% of phosphorus, about 2% of antimony and about 92% of copper.

4. A brazing alloy consisting of 6% to 7.5% of phosphorus, .5% to 2% of antimony, the combined phosphorus and antimony content ranging between 7% and 8%, and the balance substantially all copper.

PHILIP R. KALISCHER.